

March 12, 1974

J. D. CHASE

3,796,584

COLORED RUTILE BOULES AND METHOD OF MAKING THE SAME

Filed Aug. 14, 1972



INVENTOR.  
JOHN DONALD CHASE

BY

*Roland A. Dexter*

ATTORNEY

# United States Patent Office

3,796,584  
Patented Mar. 12, 1974

1

3,796,584

## COLORED RUTILE BOULES AND METHOD OF MAKING THE SAME

John Donald Chase, Stamford, Conn., assignor to American Cyanamid Company, Stamford, Conn.  
Continuation-in-part of abandoned application Ser. No. 118,748, Feb. 25, 1971. This application Aug. 14, 1972, Ser. No. 280,695  
Int. Cl. C04b 35/00, 35/46  
U.S. Cl. 106—42

2 Claims

### ABSTRACT OF THE DISCLOSURE

Single crystal rutile boules modified with both tungsten and nickel are produced which vary in color from yellow to reddish amber. The boules are produced by mixing equimolar quantities of nickel and tungsten oxides .006-0.3% NiO and 0.02-0.8% WO<sub>3</sub> by weight of TiO<sub>2</sub>, with rutile feed powder and fusing said mixture with a plasma or flame heat source to form a single crystal boule. The boules produced have potential utility as a gem material or in microwave maser applications.

The present invention relates to rutile single crystal boules. More specifically it relates to colored rutile single crystal boules and to the production of such boules. This is a continuation-in-part application of U.S. patent application Ser. No. 118,748, filed Feb. 25, 1971, now abandoned.

### BACKGROUND OF THE INVENTION

Rutile is one of the three known crystal modifications of titanium dioxide. When substantially pure, a massive single crystal of rutile has gem-like properties; with a very light straw color; and, reflectance, refraction and brilliance greater than that of diamond.

Single crystals of rutile modified or doped with transition metal ions could also be useful in semi-conductor applications. For example, one of the best materials for microwave masers in rutile doped with nickel. (L. C. Morris and D. J. Miller IEEE J. Quantum Electronics QE-1, 164, 1965.)

The preparation of colored rutile crystal boules whereby a yellow to red coloration is caused by addition of either nickel oxide or cobalt oxide is described in U.S. Pat. No. 2,715,071 or blue coloration by the addition of tungsten oxide and mixtures thereof is described in U.S. Pat. 2,801,182. However, these boules are usually significantly more difficult to grow than pure rutile due to the difficulty of incorporating the metal oxide into the rutile crystal lattice.

Although it is possible to incorporate various metal ions into a rutile crystal by the high temperature diffusion method, rather than adding the metal ions during growth, the former process involves an extra diffusion step which often requires more than 100 hours. Also, the maximum concentration of metal ion or ions added to the rutile by diffusion is less than that which can be incorporated during growth.

Rutile mixed with small quantities of two metal oxides is a commercial yellow pigment. An example of such a pigment is rutile mixed with oxides of nickel and antimony which is marketed by the Glidden Durkee Div. of S.C.M. Corporation.

### OBJECTS OF THE INVENTION

The principal object of the present invention is the preparation of rutile single crystal boules, having colors ranging from yellow to amber, which may be used as gem material. A further object of this invention is the preparation of rutile single crystal boules modified with tungsten and nickel oxides. A further object is to produce rutile

2

boules so modified with oxides of tungsten and nickel which may be used as a quantum electronic material.

### SUMMARY OF THE INVENTION

In its broadest aspects the present invention contemplates a rutile single crystal boule containing as a coloring agent the combined oxides of tungsten and nickel in substantially equimolar amounts. These colored boules are prepared according to the method of the present invention by progressively fusing a mixture of finely divided titanium dioxide and a small amount of said coloring agent mentioned above in a plasma or flame carrying an excess of an oxidizing gas to form said boule and thereafter oxidizing the boule so formed.

In this description of the present invention the word "boule" is used in its currently accepted meaning to denote a characteristic shape or form of an artificially prepared massive single crystal having a rounded end, or meniscus, a more or less rod-like body portion and a tapering end.

It has been found that rutile boules modified by additions of equal mole quantities of tungsten and nickel are easier to grow than a boule grown using a feed powder which contained a similar amount of nickel oxide, but with no tungsten oxide. The reason for the greater ease in growing rutile crystals when both nickel and tungsten are present, is postulated to be due to charge balance which is possible in the lattice when metal ions of both higher and lower valences than titanium are present. By means of the present invention rutile single crystals may be produced in various colors. Further, these large single rutile crystals modified with more than one metal oxide additive can be used for making optical measurements to evaluate various mixed oxide systems as candidates for commercial colored inorganic pigments.

Many different oxides have been separately incorporated into a rutile host crystal such as Ga<sub>2</sub>O<sub>3</sub>, CoO, NiO, Al<sub>2</sub>O<sub>3</sub>, which are described in U.S. Pats. 2,756,157, 2,715,071, 2,715,070 and Gd<sub>2</sub>O<sub>3</sub>, Eu<sub>2</sub>O<sub>3</sub>, Sm<sub>2</sub>O<sub>3</sub>, and Cr<sub>2</sub>O<sub>3</sub>, which are reported elsewhere. In all cases the melting points of these oxides have been higher than 1820° C., the melting point of the rutile host. However, in the present invention where a rutile crystal has been modified with oxides of both tungsten and nickel, the tungsten oxide, WO<sub>3</sub>, with a melting point of only 1473° C. was still retained in the boule. This was surprising, since it is normal during growth of crystals comprising several components by the Verneuil technique, for the most volatile components to distill off from the molten cap of the boule during the crystallization process. The reason for the surprising retention of WO<sub>3</sub> in the boule and thus the stability of this mixed oxide system is thought to result from the charge balance concept.

### BRIEF DESCRIPTION OF THE DRAWING

The drawing shows a comparison of the absorption coefficients for rutile and rutile modified in accordance with the invention. This modified rutile boule consists of 0.067 weight percent of NiO, 0.208 weight percent of WO<sub>3</sub> and balance is TiO<sub>2</sub>.

### DESCRIPTION OF THE INVENTION

According to the preferred method of the present invention there is employed as starting material a substantially pure TiO<sub>2</sub> powder which is very fine and uniform and is capable of being rapidly melted. A TiO<sub>2</sub> having an ultimate unit particle size of approximately 0.1 micron has proved especially satisfactory. In general, material having an average particle size above about 5 microns should be avoided because such particles do not satisfactorily fuse under the conditions of this invention. A preferred method

for preparing a feed material especially adapted for the production of rutile single crystal boules is described.

The small amount of the coloring agent, i.e., the oxides of tungsten and nickel, may be mixed with the  $TiO_2$  starting material in any convenient manner, for instance, by dry blending. A particularly suitable feed material is one where high purity (99.9 + %)  $TiO_2$  is mixed with reagent grade tungstic acid ( $H_2WO_4$ ) and reagent grade nickel nitrate hexahydrate  $Ni(NO_3)_2 \cdot 6H_2O$  in such proportions that the atomic ratios of  $Ti:W:Ni$  are present as 15:0.1:0.1. The mixture is then calcined above 700° C. and ground in a mortar to obtain a feed material of suitable consistency. Alternatively, the oxides may be made by preparing the ammonium-metal-sulphate double salt and subsequently calcining this.

The amount of coloring agent to be added to the  $TiO_2$  feed material is determined by the color desired or more precisely the location of the absorption edge within the visible spectrum. For pleasing colors and good quality boules the tungsten of the feed should not exceed 1% or about 0.3% for nickel calculated as the element based on the weight of the  $TiO_2$ . The amounts of coloring agent will vary to produce the various depths of colors and the range for each element will be subsequently described. The preferred lower limit of the feed is about 0.005% for nickel and 0.0017% for tungsten at which the boules produced possesses a light yellow color. Concentrations of coloring agents below the above lower limits result in boules substantially similar in color to plain rutile boules.

The single crystal rutile boules thereby produced have pleasing colors varying from yellow to reddish amber. This is achieved by the presence of substantially equimolar amounts of nickel oxide and tungsten oxide with the nickel oxide ranging from 0.006 to 0.3 weight percent based on the total weight of the boule. This range in turn defines the range of tungsten oxide which is from 0.02 to 0.8 weight percent. A preferred concentration of nickel oxide ranges from 0.06 to 0.07 weight percent which in turn establishes that the equimolar range of tungsten oxide is 0.19 to 0.23 weight percent for this provides a transparent, uniquely amber rutile crystal.

Another requirement of the amounts of coloring agents, i.e., nickel oxide and tungsten oxide, is that they be present in substantially equal mole quantities in the feed material in order for them to be present in the boule in this ratio. The following model is suggested to explain the increased stability of the solid solution system consisting of rutile modified with nickel and tungsten.

It is known that metal ions incorporated into a rutile crystal lattice are usually in substitutional sites. That is, they occupy the position normally occupied by titanium ions ( $Ti^{+4}$ ). In prior art, when a single metal oxide is added to a rutile boule, charge balance will not occur without defects or dislocations because the single cations have valences other than +4. For example, if charge balance was to obtain with two +2 valence metal ions then either these two ions would both have to occupy a single titanium ion substitutional site, or a defect or dislocation must occur in the lattice. Of these two possibilities, the former is unlikely since the relevant metal ion additives are quite similar in size to titanium. According to this invention, however, since two metal ions are added to the rutile lattice, one of which has a valence higher than  $Ti^{+4}$ , i.e.,  $W^{+6}$ , and the other which has a valence lower than  $Ti^{+4}$ , i.e.,  $Ni^{+2}$ , then charge compensation can occur when two titanium ions are replaced by one tungsten and one nickel ion.

In progressively fusing the starting mixture of  $TiO_2$  and oxides of nickel and tungsten, there is employed a heat source which preferably contains oxygen. The heat source can be a plasma, preferred herein, or a flame. The fusion is carried out at a temperature of from 1825° C. to 1900° C. The temperature of the gas enveloping the boule should be carefully controlled during formation of the boule.

Rutile melts at about 1820° C. and therefore it is necessary to operate so that the temperature at the top of the boule is somewhat above the melting point, e.g., 1825° C. If the temperature is in excess of 1900° C. an excessively large portion of the boule melts at the top and the molten material runs over the sides of the boule. For a plasma, argon or a similar inert gas is used as the carrier gas. In order for the plasma to be suitably oxidizing it should contain more than 2% oxygen.

Excess oxygen in the boule enveloping gas is necessary because at elevated temperatures, titanium dioxide gives up oxygen and is converted to lower, or sub-oxides of titanium, e.g.,  $Ti_2O_3$ .

Even when operating with an excess of oxygen, the boule as produced has generally a deep blue-black color indicative of some deficiency in oxygen. Therefore, in order to produce a boule according to the instant invention in which the color ranges from yellow through reddish amber, the blue-black boule has to be re-oxidized.

The reoxidation of the boule is preferably carried out by heating the blue-black boule in an oxidizing atmosphere, for instance, air or oxygen. The temperature of the treatment should be within the range from about 650° C. to about 1500° C. It has been found that at temperatures to any extent below 650° C. oxygen will not be appreciably incorporated into the rutile single crystal. There is a decided loss in brilliance, lustre and fire when the treatment is carried out above 1500° C. and at that temperature the rate of oxygen incorporated into the rutile crystal is excessively rapid and difficult to control. Preferably the oxidation should be carried out at about 1100° C. to 1475° C. to properly anneal the boule. The heating should be continued until the boule obtains the desired color, e.g., at least 60 hours at 1450° C.

According to the present invention it is necessary to fully oxidize the blue-black single crystal boule when employing the coloring agent in order to reveal the characteristic colors of such agent. When the boule is only partially oxidized the true color is masked by the blue of the oxygen deficient boule thus producing colors having bluish or greenish tone. The elements when added to  $TiO_2$  feed material produce boules having various colors. The color of the boules varies in depth and tone when the elements are present in different amounts. When any of these elements are present in the boule in very small quantities the color of the boule is yellow, varying from a pale yellow to a yellow with a brownish tone. When present in slightly larger quantities the rutile single crystal boule possesses an amber color. When present in still larger quantities the color changes from a reddish amber to almost black color.

An illustration of the quality of boules obtained from various compositions of feed powder is given in Table I. The improved boule quality resulting from the addition of both tungsten and nickel compared to that of nickel alone is shown, as is also the effect of concentration of the tungsten and nickel additives on boule color.

In order to more fully illustrate this invention the method of preparing the boule of the invention is hereafter described in the example.

TABLE I

| Addition agent                       | Amount addition agent<br>(calculated as atomic<br>ratio of metal ion in<br>feed powder) | Condition of boule               | Color (after furnace<br>oxidation) |
|--------------------------------------|-----------------------------------------------------------------------------------------|----------------------------------|------------------------------------|
| Nickel oxide.....                    | Ti:Ni=15:0.1                                                                            | Poor boule, polycrystalline..... | Yellowish brown, (opaque).         |
| Nickel oxide and tungsten oxide..... | Ti:W:Ni=15:0.1:0.1                                                                      | Good quality.....                | Yellow-amber (transparent).        |
| Do.....                              | Ti:W:Ni=15:0.5:0.5                                                                      | .....do.....                     | Amber (transparent).               |

**5**  
**EXAMPLE**

To prepare the feed material for atomic ratios of Ti:W:Ni=15:0.1:0.1, 8.56 grams of 99.95+%  $TiO_2$  (Gallard Schlesinger Co.) were mixed with 0.18 gram reagent grade  $H_2WO_4$  and 0.21 gram of reagent grade  $Ni(NO_3)_2 \cdot 6H_2O$ . This mixture was slurried in water before grinding in an electric mortar. Then the mixture was calcined for 4 hours in a furnace at 1000° C. After grinding again in the mortar the powder was screened and that which passed through a No. 70 mesh screen was used as the feed powder.

The feed powder, having an average particle size of  $0.3\mu$  and composed of mainly  $TiO_2$ , along with smaller quantities of  $WO_3$  and  $NiO$ , was fed at a constant rate of 0.05 gram/minute; suspended in an argon flow of 1 liter/minute; and passed by means of a cooled-probe through an induction plasma. The plasma gas was a mixture of 97% argon and 3% oxygen; and, was admitted at the rate of 18 l./m. to a plasma torch consisting primarily of a 28 mm. I.D. quartz tube in which power is inductively coupled to the gas, thereby cold gas and feed material entered at the back and the hot gases and feed material were expelled at the front into a 2 in. I.D., zirconia muffle. Positioned in the muffle just below the torch and enveloped by the tail flame from the plasma, the boule was located on the top of an alumina rod which was rotated and withdrawn at the boule growth rate. A sight port in the muffle allowed constant observation of the boule growth and measurement of temperature by an optical pyrometer. A  $\frac{3}{4}$  in. long boule, of diameter which varied from  $\frac{1}{8}$  in. at the bottom to  $\frac{1}{2}$  in. at the top, was grown over a period of 4 hours. The as-grown boule was black in color. After growing the boule it was oxidized for 65 hours at 1425° C. in a tube furnace. The oxidized boule was a yellow-amber color. A 1 millimeter thick slab, cut from the boule and polished, was transparent and consisted of 0.067 weight percent of  $NiO$ , 0.208 weight percent of  $WO_3$  and balance of  $TiO_2$ .

In order to show the effect of the addition of nickel and tungsten oxide to rutile, the measured absorption coefficient of the boule of the example is plotted in the drawing for the visible region of the spectrum and compared with a pure rutile crystal. The absorption edge is seen to be shifted about 500 Å. to longer wavelengths and toward the red end of the visible spectrum, and a residual absorption about 100 times greater than that of rutile was imparted to the boule by the nickel and tungsten oxides.

**6**

From the above description it has been shown that pleasant appearing colored rutile boules may be formed by the present invention. The coloring agents produce products which range in color from yellow through amber to reddish-black tones when added in varying quantities. The precise depth of tone and nature of the color obtained is readily controlled as hereinbefore described by employment of the appropriate mixture. These colored boules may be cut into gems which possess the required characteristics, particularly that of hardness and a pleasing appearance, which are necessary for the gem trade. They may also have application as a quantum electronic material, for example, a microwave maser.

While this invention has been described and illustrated by the example shown, it is not intended to be strictly limited thereto and other modifications and variations may be employed within the scope of the following claims.

I claim:

1. A colored rutile single crystal boule containing oxides of tungsten and nickel in substantially equimolar amounts wherein said  $WO_3$  content ranges from 0.02 to 0.8 percent and said  $NiO$  content ranges from 0.006 to 0.3 percent by weight based on said boule.

2. The boule of claim 1 wherein said  $WO_3$  content ranges from 0.19 to 0.23 percent and said  $NiO$  content ranges from 0.06 to 0.07 percent.

**References Cited**

**UNITED STATES PATENTS**

|    |           |        |        |       |        |
|----|-----------|--------|--------|-------|--------|
| 30 | 2,715,071 | 8/1955 | Merker | ----- | 106—42 |
|    | 2,801,182 | 7/1957 | Merker | ----- | 106—42 |
|    | 2,715,070 | 8/1955 | Moore  | ----- | 106—42 |
|    | 3,558,333 | 1/1971 | Beals  | ----- | 106—42 |

**FOREIGN PATENTS**

|    |         |        |               |       |        |
|----|---------|--------|---------------|-------|--------|
| 25 | 686,490 | 1/1953 | Great Britain | ----- | 106—42 |
|----|---------|--------|---------------|-------|--------|

**OTHER REFERENCES**

40 Johnson, G., et al.: "Influence of Minor Additions on Color and Electrical Properties of Rutile," J. Am. Cer Soc. 32 (1949), pp. 398—401.

HELEN M. McCARTHY, Primary Examiner

U.S. Cl. X.R.

23—301

UNITED STATES PATENT OFFICE  
CERTIFICATE OF CORRECTION

Patent No. 3,796,584 Dated March 20, 1974

Inventor(s) CHASE, JOHN DONALD

It is certified that error appears in the above-identified patent and that said Letters Patent are hereby corrected as shown below:

Column 1, line 39, after the word masers, change "in" to -- is --.

Column 3, line 16, after the word amount, change "if" to -- of --.

Signed and sealed this 23rd day of July 1974.

(SEAL)  
Attest:

McCOY M. GIBSON, JR.  
Attesting Officer

C. MARSHALL DANN  
Commissioner of Patents